

# United States Patent [19]

Fang et al.

[11] Patent Number: 4,924,074

[45] Date of Patent: May 8, 1990

[54] ELECTRICAL DEVICE COMPRISING CONDUCTIVE POLYMERS

[75] Inventors: **Shou-Mean Fang**, Union City; **Charles H. Camphouse**, Mountain View, both of Calif.

[73] Assignee: **Raychem Corporation**, Menlo Park, Calif.

[21] Appl. No.: 293,542

[22] Filed: Jan. 3, 1989

### Related U.S. Application Data

[63] Continuation of Ser. No. 103,077, Sep. 30, 1987, abandoned.

[51] Int. Cl.<sup>5</sup> ..... H05B 3/10

[52] U.S. Cl. ..... 219/548; 219/541; 219/549; 219/553; 338/22 SD

[58] Field of Search ..... 338/20, 22 R, 22 SD, 338/26; 219/548, 541, 544, 549, 552, 553; 156/85

### References Cited

#### U.S. PATENT DOCUMENTS

|           |         |                        |          |
|-----------|---------|------------------------|----------|
| 3,243,753 | 3/1966  | Kohler et al.          | 338/31   |
| 3,351,882 | 11/1967 | Kohler et al.          | 338/322  |
| 3,861,029 | 1/1975  | Smith-Johannsen et al. | 29/611   |
| 4,177,376 | 12/1979 | Horsma et al.          | 219/553  |
| 4,237,441 | 12/1980 | van Konynenburg et al. | 338/22 R |
| 4,238,812 | 12/1980 | Middleman et al.       | 361/106  |
| 4,272,471 | 6/1981  | Walker                 | 264/104  |
| 4,286,376 | 9/1981  | Smith-Johannsen et al. | 29/611   |
| 4,317,027 | 2/1982  | Middleman et al.       | 219/553  |
| 4,327,351 | 4/1982  | Walker                 | 338/22 R |
| 4,329,726 | 5/1982  | Middleman et al.       | 361/58   |
| 4,330,703 | 5/1982  | Horsma et al.          | 219/553  |
| 4,352,083 | 9/1982  | Middleman et al.       | 338/23   |

|           |         |                  |          |
|-----------|---------|------------------|----------|
| 4,388,607 | 6/1983  | Toy et al.       | 338/22   |
| 4,400,614 | 8/1983  | Sopory           | 219/528  |
| 4,413,301 | 11/1983 | Middleman et al. | 361/106  |
| 4,426,633 | 1/1984  | Taylor           | 338/25   |
| 4,445,026 | 4/1984  | Walker           | 219/553  |
| 4,481,498 | 11/1984 | McTavish et al.  | 338/20   |
| 4,514,620 | 4/1985  | Cheng et al.     | 219/553  |
| 4,542,365 | 9/1985  | McTavish et al.  | 338/20   |
| 4,543,474 | 9/1985  | Horsma et al.    | 219/553  |
| 4,549,161 | 10/1985 | McTavish et al.  | 338/20   |
| 4,654,511 | 3/1987  | Horsma et al.    | 219/548  |
| 4,689,475 | 8/1987  | Matthiesen       | 219/553  |
| 4,724,417 | 2/1988  | Au et al.        | 338/22 R |
| 4,743,321 | 5/1988  | Soni et al.      | 156/85   |

### FOREIGN PATENT DOCUMENTS

|         |         |                      |
|---------|---------|----------------------|
| 0038713 | 10/1981 | European Pat. Off.   |
| 098647  | 1/1984  | European Pat. Off.   |
| 063440  | 6/1987  | European Pat. Off.   |
| 2434006 | 2/1976  | Fed. Rep. of Germany |
| 2644256 | 3/1978  | Fed. Rep. of Germany |
| 7623707 | 8/1976  | France               |
| 2528253 | 12/1983 | France               |

Primary Examiner—E. A. Goldberg

Assistant Examiner—M. M. Lateef

Attorney, Agent, or Firm—Marguerite E. Gerstner; Timothy H. P. Richardson; Herbert G. Burkard

### ABSTRACT

A process for preparing an electrical device which has a conductive polymer exhibiting PTC behavior. The cross-linking may be to a level of 50 to 100 Mrad or higher for devices designed to withstand high voltage test conditions. The device may be a laminar device having a center layer of higher resistivity than two surrounding layers.

20 Claims, 1 Drawing Sheet





*FIG\_1*

## ELECTRICAL DEVICE COMPRISING CONDUCTIVE POLYMERS

### CROSS-REFERENCE TO RELATED APPLICATIONS

This application is a file wrapper continuation of copending application Ser. No. 103,077 (Fang et al) filed Sept. 30, 1987 now abandoned. This application is also related to copending application Ser. No. 102,987 (Fang et al) filed Sept. 30, 1987. The entire disclosure of each of these applications is incorporated herein by reference.

### BACKGROUND OF THE INVENTION

#### 1. Field of the Invention

This invention relates to electrical devices comprising conductive polymer compositions.

#### 2. Introduction to the Invention

Conductive polymer compositions exhibiting PTC behavior, and electrical devices comprising them, are well known. Such electrical devices may comprise circuit protection devices, self-regulating strip heaters, or elongate cathodic protection devices. Reference may be made, for example, to U.S. Pat. Nos. 4,177,376, 4,330,703, 4,543,474 and U.S. Pat. No. 4,654,511 (Horsma, et al.), U.S. Pat. No. 4,237,441 (van Konynenburg, et al.), U.S. Pat. Nos. 4,238,812 and 4,329,726 (Middleman, et al.), U.S. Pat. No. 4,352,083 (Middleman, et al.), U.S. Pat. No. 4,317,027 (Middleman, et al.), U.S. Pat. No. 4,426,633 (Taylor), U.S. Pat. No. 3,351,882 (Kohler, et al.), U.S. Pat. No. 3,243,753 (Kohler), U.S. Pat. No. 4,689,475 (Matthiesen), U.S. Pat. Nos. 3,861,029 and 4,286,376 (Smith-Johannsen, et al.), French Patent Application No. 76 23707 (Moyer), and commonly assigned, copending applications, Ser. Nos. 141,989 (MP0715, Evans), 656,046 (MP0762, Jacobs, et al.), abandoned in favor of a file wrapper continuation Ser. No. 146,460 (filed Jan. 21, 1988) and published as European Patent Application No. 63,440, Ser. No. 051,438 (MP0897-US5, Batliwalla, et al.) now U.S. Pat. No. 4,761,541, and Ser. No. 711,910 (MP1044, Au, et al.) now U.S. Pat. No. 4,724,417. The disclosure of each of the patents, publications, and applications referred to above is incorporated herein by reference.

Electrical devices with improved physical properties and improved electrical performance are achieved when the conductive polymer composition comprising the device is crosslinked. Such cross-linking can be accomplished through the use of chemical cross-linking agents or gamma or electron irradiation, or a combination of these. It is frequently true that ionizing irradiation generated by an electron beam results in the most rapid and cost-effective means of cross-linking.

### SUMMARY OF THE INVENTION

We have discovered that one difficulty with this type of irradiation is the rapid temperature rise in the conductive polymer as a result of irradiation to high doses. An additional problem is that under these conditions, 60 gases are generated during the cross-linking process more rapidly than they can be dissipated. This is particularly true for polymers that are irradiated to levels in excess of 50 or 100 Mrad, designed for use as circuit protection devices under conditions of high voltage. Such devices have been made with parallel columnar electrodes embedded in the conductive polymer matrix, rather than laminar metal foil or mesh electrodes at-

tached to the surface of the conductive polymer element because of the delamination of the metal foil electrodes as a result of the gases generated. For instance, U.S. Ser. No. 656,046, now abandoned in favor of a file 5 wrapper continuation Ser. No. 146,460, that it is necessary to irradiate a laminar polymer element before the laminar electrodes are attached to form a device. For devices comprising embedded columnar electrodes, rapid heating and generation of gases during irradiation may result in the formation of voids at the polymer/electrode interface, producing contact resistance and sites for electrical failure during operation at high voltages.

In order to efficiently and cheaply manufacture electrical devices it is desirable that laminar metal foil electrodes be attached prior to irradiation and that devices with columnar electrodes do not suffer from void-formation at the polymer/electrode interface as a result of rapid gas generation. It is also desirable that a laminar device be capable of withstanding relatively high voltages and currents without delamination of the laminar electrodes. We have found that electrical devices with improved performance can be produced if the conductive polymer element is maintained at a low temperature during the irradiation process.

Accordingly, in its first aspect, this invention provides a process for the preparation of an electrical device which comprises

- (1) a PTC element composed of a cross-linked conductive polymer composition which exhibits PTC behavior and which comprises a polymeric component and, dispersed in the polymeric component, a particulate conductive filler; and
  - (2) two electrodes which are electrically connected to the PTC element and which are connectable to a source of electrical power to cause current to pass through the PTC element,
- which process comprises subjecting the PTC element to radiation cross-linking in which
- (i) said cross-linking is achieved by use of an electron beam;
  - (ii) said cross-linking is conducted such that the radiation dose absorbed by each current-carrying part of the PTC element is at least 50 Mrad; and
  - (iii) during the cross-linking process, no part of the PTC element which is in contact with the electrodes reaches a temperature greater than  $(T_m - 60)^\circ\text{C}$ , where  $T_m$  is the temperature measured at the peak of the endothermic curve generated by a differential scanning calorimeter for the lowest melting polymer in the polymeric component.

We have also discovered that improved laminar electrical devices comprise

- (1) a laminar PTC element; and
- (2) two laminar equidistant electrodes which are adjacent to and in electrical contact with said laminar PTC element; said PTC element comprising
  - (a) a first layer which is composed of a first conductive polymer composition,
  - (b) a second layer which is composed of a second conductive polymer composition, and
  - (c) a third layer which is composed of a third conductive polymer composition;

and in which the first, second and third layers are arranged so that all current paths between the electrodes pass sequentially through the first, second and third layers; the resistivity of the second composition at  $23^\circ\text{C}$

C. is higher than the resistivity of the first composition at 23° C. and higher than the resistivity of the third composition at 23° C.; and each of the conductive polymer compositions comprises a polymeric component and, dispersed in the polymeric component, a particulate conductive filler; and at least one of the following conditions is present

- (i) each of the first and third compositions exhibits PTC behavior with a switching temperature which is within 15 degrees of the switching temperature of the second composition;
- (ii) the average thickness of the second layer is less than 33% of the distance between the electrodes;
- (iii) the resistivity of the second composition is less than 50 ohm-cm;
- (iv) the resistance of the second layer is less than 100 ohms; and
- (v) the resistivity of each of the first and third compositions at 23° C. is less than 0.1 times the resistivity of the second composition at 23° C.

#### BRIEF DESCRIPTION OF THE DRAWINGS

The invention is illustrated in the accompanying drawing in which FIG. 1 shows an electrical device of the invention in plan view.

#### DETAILED DESCRIPTION OF THE INVENTION

The invention described herein concerns electrical devices comprising a conductive polymer element and processes for preparing such devices. The conductive polymer element is composed of a polymeric component and, dispersed in the polymeric component, a particulate conductive filler. The polymeric component is preferably a crystalline organic polymer or blend comprising at least one crystalline organic polymer, such term being used to include siloxanes. The polymeric component has a melting temperature which is defined as the temperature at the peak of the endothermic curve generated by a differential scanning calorimeter. If the polymeric component is a blend of polymers, the melting temperature is defined as the melting temperature of the lowest melting polymeric component. The conductive filler may be graphite, carbon black, metal, metal oxide, or a combination of these. The conductive polymer element may also comprise antioxidants, inert fillers, prorads, stabilizers, dispersing agents, or other components. Dispersion of the conductive filler and other components may be conducted by dry-blending, melt-processing or sintering. The resistivity of the conductive polymer is measured at 23° C. (i.e. room temperature).

The conductive polymer element exhibits PTC behavior with a switching temperature,  $T_s$ , defined as the temperature at the intersection of the lines drawn tangent to the relatively flat portion of the log resistivity vs. temperature curve below the melting point and the steep portion of the curve. Suitable compositions are disclosed in the references cited. If the PTC element comprises more than one layer, and one or more of the layers is made of a polymeric composition that does not exhibit PTC behavior the composite layers of the element must exhibit PTC behavior.

The electrical device has two electrodes which are electrically connected to the PTC element and which are connectable to a source of electrical power to cause current to pass through the PTC element. The electrodes may be parallel columnar wires embedded within

the conductive polymer or laminar electrodes comprised of metal foil or mesh and attached to the surface of the PTC element. Particularly preferred are metal foil electrodes of nickel or copper with an electrodeposited layer that has a microrough surface.

The electrical device may be cross-linked by the use of a chemical cross-linking agent or a source of ionizing radiation, such as a cobalt source or an electron beam. Electron beams are particularly preferred for efficiency, speed, and cost of irradiation. The devices may be irradiated to any level, although for devices intended for use in high voltage applications, doses of 50 to 100 Mrad or more (e.g. to 150 Mrad) are preferred. The irradiation may be conducted in one step or in more than one step; each irradiation segment may be separated by a heat-treatment step in which the PTC element is heated to a temperature above the melting point of the polymeric component and is then cooled to recrystallize the polymeric component. The cross-linking process may be conducted with or without the electrodes attached to the PTC element. The radiation dose is defined as the minimum amount of radiation dose absorbed by each current-carrying part of the PTC element. In the case of laminar electrical devices in which the current flows in a direction normal to the plane of the laminar electrode (i.e. through the thickness of the PTC element), the entire PTC element must be irradiated to the minimum dose. For devices with embedded columnar electrodes, the center of the PTC element, between and parallel to the electrodes, must be irradiated to the minimum dose.

It is preferred that during the irradiation step, the temperature of no part of the PTC element which is in contact with the electrodes reaches a temperature greater than  $(T_m - 60)^\circ\text{C}$ ., particularly  $(T_m - 80)^\circ\text{C}$ . In the case of devices composed of high density polyethylene which has a  $T_m$  of about  $130^\circ\text{C}$ ., it is preferred that the temperature remain less than  $60^\circ\text{C}$ ., particularly less than  $50^\circ\text{C}$ ., especially less than  $40^\circ\text{C}$ . In the case of an electron beam, this may be accomplished by cooling the devices through the use of fans or gas, or positioning the devices next to objects with large heat-sinking capabilities. It has been observed that if the device remains cool during the irradiation process the rate of gas generation (i.e. hydrogen from the cross-linking step) is balanced by the rate of diffusion of the gas from the device and few, if any, bubbles are observed at the interface of the PTC element and the electrodes. The result is that, in the case of laminar devices, the laminar electrodes do not delaminate, and with embedded columnar electrodes, the number and frequency of bubbles or voids at the polymer/electrode interface is limited. This results in improved electrical performance during application of electrical current.

Laminar electrical devices of the invention may comprise PTC elements which comprise three or more layers of conductive polymer. The layers may have the same or a different polymeric component or the same or a different conductive filler. Particularly preferred are devices with first, second and third layers arranged so that all current paths between the electrodes pass sequentially through the first, second and third layers. It is desirable that the second layer, which is sandwiched between the first and third layers, is the site of the hot-line which is formed when the device is exposed to an electrical current. This can be achieved by the use of a second layer which has a room temperature resistivity higher than that of both the first and the third layers.

During operation, through  $I^2R$  heating, heat will be generated at the site of the highest resistance; this process will be enhanced by the limited thermal dissipation of the center region (second layer) of the device with respect to the top or bottom regions (first or third layers). If the hot line is controlled at the center of the device, it will not form at the electrodes, eliminating one failure mechanism common to laminar devices.

The resistivity of the three layers can be varied in several ways. The polymeric component of the layers may be the same, but the volume loading of conductive filler can be different for the second layer. In most cases, a higher resistivity is achieved by the use of either a lower volume loading of conductive filler or the same loading of a conductive filler with a lower electrical conductivity than the filler of the first layer. In some cases, a higher resistivity can be achieved by the use of the same volume loading of conductive filler but a lower loading of a non-conductive filler. It has been found that when the conductive filler is carbon black, useful compositions can be achieved when the polymeric component is the same for the layers, but the carbon black loading of the second layer is at least 2, preferably at least 3, especially at least 4 volume percent lower than that of the first or third layers. The resistivity of the second layer is preferably at least 20 percent, particularly at least two times, especially at least five times higher than the resistivity of the first and third layers. A PTC element made from the three layers may have a second layer with a resistivity of less than 50 ohm-cm or a resistance of less than 100 ohms. In another embodiment, the resistivity of the first layer and the third layer is less than 0.1 times the resistivity of the second layer.

Layered devices have been disclosed in the art for constructions of PTC and ZTC materials which differ in resistivity by at least one order of magnitude. It has been found that useful laminar devices can be made where all three layers exhibit PTC behavior if the switching temperature,  $T_s$ , of each of the layers is within 15° C. of the switching temperature of the second layer. It is preferred that  $T_s$  be the same for all three layers; this can be achieved by the use of the same polymeric component in the conductive polymer composition for each layer.

Useful layered laminar devices with hotline control can also be made when the second layer comprises less than one-third, preferably less than one-fourth, particularly less than one-fifth of the total thickness of the first, second and third layers. Preferred devices have a total thickness of at least 0.060 inch, particularly at least 0.100 inch. They have a resistance of less than 100 ohms. Such devices are useful for circuit protection applications where the applied voltage is 120 V or greater, particularly when they have been exposed to irradiation to a level of more than 50 Mrad.

Referring now to the Figure, FIG. 1 shows an electrical device (specifically a circuit protection device) 1 which has two laminar metal electrodes 10, 10' attached to a PTC element 20. The PTC element is composed of a first conductive polymer layer 21 and a third conductive polymer layer 23 sandwiching a second conductive polymer layer 22.

We claim:

1. A process for the preparation of an electrical device which comprises

(1) a PTC element composed of a cross-linked conductive polymer composition which exhibits PTC

behavior and which comprises a polymeric component and, dispersed in the polymeric component, a particulate conductive filler; and

(2) two electrodes which are electrically connected to the PTC element and which are connectable to a source of electrical power to cause current to pass through the PTC element,

which process comprises subjecting the PTC element to radiation cross-linking in which

- (i) said cross-linking is achieved by use of an electron beam;
- (ii) said cross-linking is conducted such that the radiation dose absorbed by each current-carrying part of the PTC element is at least 50 Mrad; and
- (iii) during the cross-linking process, no part of the PTC element which is in contact with the electrodes reaches a temperature greater than  $(T_m - 60)^\circ\text{C}$ , where  $T_m$  is the temperature measured at the peak of the endothermic curve generated by a differential scanning calorimeter for the lowest melting polymer in the polymeric component.

2. A process claim 1 wherein the minimum radiation dose is at least 100 Mrad.

3. A process according to claim 1 wherein the minimum radiation dose is at least 150 Mrad.

4. A process according to claim 1 wherein said cross-linking is conducted in two steps, said steps being separated by a heat-treatment process wherein said PTC element is heated to a temperature above the melting temperature of the polymeric component and is then cooled to recrystallize the polymer.

5. A process according to claim 1 wherein said electrodes comprise electrodeposited metal foil and said electrodes are attached to said PTC element prior to said radiation-crosslinking.

6. An electrical device which comprises:

- (1) a laminar PTC element; and
- (2) two laminar equidistant electrodes which are adjacent to and in electrical contact with said laminar PTC element; said PTC element comprising
  - (a) a first layer which is composed of a first conductive polymer composition,
  - (b) a second layer which is composed of a second conductive polymer composition, and
  - (c) a third layer which is composed of a third conductive polymer composition;

and in which the first, second and third layers are arranged so that all current paths between the electrodes pass sequentially through the first, second and third layers; the resistivity of the second composition at 23° C. is higher than the resistivity of the first composition at 23° C. and higher than the resistivity of the third composition at 23° C.; and each of the conductive polymer compositions comprises a polymeric component and, dispersed in the polymeric component, a particulate conductive filler; at least one of the following conditions is present

- (i) each of the first and third compositions exhibits PTC behavior with a switching temperature which is within 15° C. of the switching temperature of the second composition;
- (ii) the average thickness of the second layer is less than 33% of the distance between the electrodes;
- (iii) the resistivity of the second composition at 23° C. is less than 50 ohm-cm;
- (iv) the resistance of the second layer is less than 100 ohms; and

(v) the resistivity of each of the first and third compositions 23° C. is less than 0.1 times the resistivity of the second composition at 23° C.

7. A device according to claim 6 wherein said first, second and third compositions comprise the same polymeric component.

8. A device according to claim 7 wherein said first, second and third compositions comprise the same particulate conductive filler.

9. A device according to claim 8 wherein said particulate conductive filler comprises carbon black.

10. A device according to claim 8 wherein the second composition comprises a lower volume loading of carbon black and a lower volume loading of nonconductive filler than each of the first and third compositions.

11. A device according to claim 10 wherein the carbon black loading in the second composition is at least 2 volume percent lower than that in the first and third compositions.

12. A device according to claim 10 wherein the carbon black loading in the second composition is at least 4 volume percent lower than that in the first and third compositions.

13. A device according to claim 6 wherein the resistivity at 23° C. of the second composition is at least 20 percent higher than the resistivity at 23° C. of the first and third compositions.

14. A device according to claim 6 wherein the resistivity at 23° C. of the second composition is at least two times the resistivity at 23° C. of the first and third compositions.

15. A device according to claim 6 wherein the resistivity at 23° C. of the second composition is at least five times the resistivity at 23° C. of each of the first and third compositions.

16. A device according to claim 6 wherein the thickness of the laminar PTC element is at least 0.060 inch.

17. A device according to claim 6 wherein the thickness of the laminar PTC element is at least 0.100 inch.

18. A device according to claim 6 wherein said second layer is a ZTC layer.

19. A device according to claim 6 wherein the resistance of the device is less than 100 ohms.

20. A device according to claim 6 wherein the electrodes have a surface of electrodeposited nickel.

\* \* \* \* \*